

1

3,734,733  
**POSITIVE WORKING PHOTO-THERMOGRAPHIC MATERIALS CONTAINING BI-IMIDAZOLYL COMPOUNDS AND REDUCING AGENTS AND THE USE THEREOF IN COLOR DEVELOPMENT**

Albert Lucien Poot, Kontich, Jan Frans van Besauw, Brasschaat, and Theofiel Hubert Ghys, Kontich, Belgium, assignors to Agfa-Gevaert N.V., Mortsel, Belgium  
No Drawing. Filed Apr. 8, 1971, Ser. No. 132,612  
Claims priority, application Great Britain, Apr. 9, 1970, 16,998/70

Int. Cl. G03c 5/24, 1/00  
U.S. Cl. 96—48 HD 19 Claims

**ABSTRACT OF THE DISCLOSURE**

A recording element carrying a photo-oxidizing bi-imidazolyl compound in chemically reactive contact with a compound having reducing properties is imagewise exposed to activating radiation to effect reaction between the bi-imidazolyl compound in the exposed areas of the element and the reducing compound to destroy the reducing properties of the latter in such exposed areas and thereafter the exposed element is uniformly contacted with an image-forming compound which is reactive on heating with said reducing compound to produce a distinctive coloration and heated so as to produce by such reaction a visible image corresponding to the unexposed areas of the recording element.

The present invention relates to a photothermographic reproduction system and to materials used therefor.

In a well known thermographic process a heat-sensitive copy sheet is used, which when heated beyond a certain temperature, turns black or dark coloured. In the process wherein such a copy sheet is used, the original that contains infrared light-absorbing image areas is exposed to infrared radiation while being in heat-conductive contact with the copy sheet. In correspondence with the image areas of the original the copy sheet reaches a temperature at which a coloured product is formed. So, in this process heat is accumulated image-wise in the original and transferred therefrom to the copy sheet.

As there is no neutralizing action of the reactive components still present in the non-heated portions of the recording layer, the copy paper will remain heat-sensitive and the image-containing copy paper will be blackened completely by overall heating. This characteristic and the fact that this process is limited to the copying of originals containing infrared radiation-absorbing image markings on an infrared radiation-reflecting background, make that process less attractive.

In order to find a solution for the disadvantages of said process a photothermographic process has been developed as described, e.g., in the U.S. patent specification 3,094,417 of Wesley R. Workmans, issued June 18, 1968.

In the latter process the difficulty of colour-insensibility and of image stabilization of the copy sheet is solved. In said process light and heat energy are used and therefore it is called a dual one.

According to an embodiment of said process an intermediate U.V. light-sensitive sheet is used for the information-wise exposure. The intermediate sheet includes a volatilizable reductor that becomes transformed with the

2

aid of exposed photoreducible dye into a form that is unreactive for a reducible substance contained in a receptor sheet.

The present invention provides a novel photographic composition containing a photosensitive substance that by exposure to activating electromagnetic radiation destroys the reducing character of particular reducing compounds. Said photosensitive substance being a photo-oxidant is suited for being applied in a recording process, wherein in a first step information-wise modulated electromagnetic radiation is used to transform a transferable reducing agent into an unreactive species for a reducible substance, that is capable of yielding in a reaction with said reducing agent a product differing in colour from the reactants, and in a second step overall applied heat is used to transfer unmodified transferable reducing agent to a receptor layer or sheet containing said reducible substance.

The photosensitive compound used according to the present invention corresponds to the following general formula:



wherein:

each of R<sub>1</sub>, R<sub>2</sub> and R<sub>3</sub> stands for a carbocyclic or heterocyclic group with aromatic character and each dotted line circle stands for 4 delocalized electrons.

The R<sub>1</sub>, R<sub>2</sub> and R<sub>3</sub> groups having an aromatic character are e.g. a phenyl, biphenyl, naphthyl, furyl or thiényl group including said groups in substituted form. The substituents on said groups are restricted to substituents having no Zerewitinoff hydrogen atoms, in other words do not contain hydrogen atoms that are reactive with respect to methylmagnesium iodide.

Preferred bi-imidazolyl compounds correspond to the following general formula:



wherein the valencies of the atoms in the imidazolyl rings, other than those through which the imidazolyl rings are joined, are satisfied by two conjugated intracyclic double bonds, and wherein A is a substituted phenyl radical of the formula:



wherein R<sub>1</sub> represents a substituent not containing an active hydrogen atom and R<sub>2</sub>, R<sub>3</sub> and R<sub>4</sub> represent hydrogen or substituents free from active hydrogen atoms and where two of R<sub>1</sub>, R<sub>2</sub>, R<sub>3</sub> and R<sub>4</sub> in adjacent positions on the phenyl ring taken together may form a benzo ring, preferably the substituent or substituents ortho to the

imidazolyl radical having a sigma constant below 0.7; and B and D are phenyl groups which are unsubstituted or substituted with up to three substituents free from active hydrogen atoms, two of which, in adjacent positions on the phenyl ring, may together form a benzo ring; preferably at least one of the ortho positions in each of the phenyl groups B and D is unsubstituted.

The groups B and D can be alike or different as will be shown more fully below. A discussion and explanation of the sigma value is given by H. H. Jaffe in Chem. Rev. 10 53, 191 (1953), particularly pages 219 to 223.

The substituents which are free from active hydrogen atoms include alkyl, alkoxy, alkoxy-carbonyl, alkylthio, dialkylamino, dialkylcarbamoyl, dialkylsulphamoyl, alkanoyloxy, N-alkylalkanamido, aryl, aryloxy, arylthio, 15 benzo, halo, and cyano groups. The alkyl substituents and the alkyl groups of the alkoxy substituents can be of any chain length, but are preferably lower alkyls such as methyl, ethyl, propyl, butyl, isobutyl, sec.-butyl, tert.-butyl, pentyl, isopentyl. The alkanoyl and alkanamido substituents preferably contain from 1 to 6 carbon atoms, i.e. ranging from formyl to caprooyl and ranging from formamido to caproamide, respectively. The aryl groups include phenyl, 1-naphthyl, 2-naphthyl and the halo substituents include bromine, chlorine and fluorine.

Particularly preferred compounds for use according to this invention are represented by the formula:

TABLE I

| Number of the compound | R <sub>1</sub>                                   | R <sub>2</sub>                                   | R <sub>3</sub>                                   |
|------------------------|--------------------------------------------------|--------------------------------------------------|--------------------------------------------------|
| 1                      | o-Acetoxyphenyl                                  | o-Acetoxyphenyl                                  | o-Acetoxyphenyl                                  |
| 2                      | o-Benzylphenyl                                   | o-Benzylphenyl                                   | o-Benzylphenyl                                   |
| 3                      | 2,3-benzo(1-naphthyl)phenyl                      | 2,3-benzo(1-naphthyl)phenyl                      | 2,3-benzo(1-naphthyl)phenyl                      |
| 4                      | 2,3-benzophenyl                                  | 2,3-benzophenyl                                  | 2,3-benzophenyl                                  |
| 5                      | do                                               | p-Methoxyphenyl                                  | p-Methoxyphenyl                                  |
| 6                      | 3,4-benzo-2-methoxy(2-[1-methoxy]naphthyl)phenyl | 3,4-benzo-2-methoxy(2-[1-methoxy]naphthyl)phenyl | 3,4-benzo-2-methoxy(2-[1-methoxy]naphthyl)phenyl |
| 7                      | 4,5-benzo-2-methoxy(2-[3-methoxy]naphthyl)phenyl | 4,5-benzo-2-methoxy(2-[3-methoxy]naphthyl)phenyl | 4,5-benzo-2-methoxy(2-[3-methoxy]naphthyl)phenyl |
| 8                      | o-Benzylthiophenyl                               | o-Benzylthiophenyl                               | o-Benzylthiophenyl                               |
| 9                      | o-Bromophenyl                                    | o-Bromophenyl                                    | o-Bromophenyl                                    |
| 10                     | do                                               | p-Bromophenyl                                    | p-Bromophenyl                                    |
| 11                     | do                                               | o-Methoxyphenyl                                  | o-Methoxyphenyl                                  |
| 12                     | 2-bromo-4-phenyl                                 | 2-bromo-4-phenyl                                 | 2-bromo-4-phenyl                                 |
| 13                     | o-Butoxyphenyl                                   | o-Butoxyphenyl                                   | o-Butoxyphenyl                                   |
| 14                     | o-tert.Butoxyphenyl                              | o-tert.Butoxyphenyl                              | o-tert.Butoxyphenyl                              |
| 15                     | o-tert.Butylphenyl                               | o-tert.Butylphenyl                               | o-tert.Butylphenyl                               |
| 16                     | do                                               | p-tert.Butylphenyl                               | p-tert.Butylphenyl                               |
| 17                     | N-butyacetamidephenyl                            | N-butyacetamidephenyl                            | N-butyacetamidephenyl                            |
| 18                     | o-Butylthiophenyl                                | o-Butylthiophenyl                                | o-Butylthiophenyl                                |
| 19                     | o-Butyryloxyphenyl                               | o-Butyryloxyphenyl                               | o-Butyryloxyphenyl                               |
| 20                     | o-Chlorophenyl                                   | o-Chlorophenyl                                   | o-Chlorophenyl                                   |
| 21                     | do                                               | p-Chlorophenyl                                   | p-Chlorophenyl                                   |
| 22                     | do                                               | 3,4-dichlorophenyl                               | 3,4-dichlorophenyl                               |
| 23                     | do                                               | m-Pentylxylophenyl                               | m-Pentylxylophenyl                               |
| 24                     | do                                               | do                                               | Do.                                              |
| 25                     | do                                               | p-Propionyloxyphenyl                             | p-Propionyloxyphenyl                             |
| 26                     | 2-chloro-4-phenyl                                | 2-chloro-4-phenyl                                | 2-chloro-4-phenyl                                |
| 27                     | o-Cyanophenyl                                    | o-Cyanophenyl                                    | o-Cyanophenyl                                    |
| 28                     | do                                               | p-tert.Butylphenyl                               | p-tert.Butylphenyl                               |
| 29                     | do                                               | p-Cyanophenyl                                    | p-Cyanophenyl                                    |
| 30                     | do                                               | p-Methoxyphenyl                                  | p-Methoxyphenyl                                  |
| 31                     | 2,3,4,5-dibenzo(9-phenanthryl)phenyl             | 2,3,4,5-dibenzo(9-phenanthryl)phenyl             | 2,3,4,5-dibenzo(9-phenanthryl)phenyl             |
| 32                     | 2,3-dibromophenyl                                | 2,3-dibromophenyl                                | 2,3-dibromophenyl                                |
| 33                     | 2,4-dibromophenyl                                | 2,4-dibromophenyl                                | 2,4-dibromophenyl                                |
| 34                     | 2,6-dibutylphenyl                                | 2,6-dibutylphenyl                                | 2,6-dibutylphenyl                                |
| 35                     | 2,4-di-tert.butylphenyl                          | 2,4-di-tert.butylphenyl                          | 2,4-di-tert.butylphenyl                          |
| 36                     | do                                               | 2,4-difluorophenyl                               | 2,4-difluorophenyl                               |
| 37                     | do                                               | p-Fluorophenyl                                   | p-Fluorophenyl                                   |
| 38                     | o-Dibutylsulfamylphenyl                          | o-Dibutylsulfamylphenyl                          | o-Dibutylsulfamylphenyl                          |
| 39                     | 2,4-dichlorophenyl                               | 2,4-dichlorophenyl                               | 2,4-dichlorophenyl                               |
| 40                     | do                                               | o-Bromophenyl                                    | o-Bromophenyl                                    |
| 41                     | 2,4-dicyanophenyl                                | p-Cyanophenyl                                    | p-Cyanophenyl                                    |
| 42                     | 2,6-dicyanophenyl                                | 2,6-dicyanophenyl                                | 2,6-dicyanophenyl                                |
| 43                     | 2,4-diethoxyphenyl                               | 2,4-diethoxyphenyl                               | 2,4-diethoxyphenyl                               |
| 44                     | o-Diethylsulfamylphenyl                          | o-Diethylsulfamylphenyl                          | o-Diethylsulfamylphenyl                          |
| 45                     | 2,5-difluorophenyl                               | p-Cyanophenyl                                    | p-Cyanophenyl                                    |
| 46                     | do                                               | do                                               | Do.                                              |
| 47                     | 2,3-dimethoxyphenyl                              | 2,3-dimethoxyphenyl                              | 2,3-dimethoxyphenyl                              |
| 48                     | 2,4-dimethoxyphenyl                              | 2,4-dimethoxyphenyl                              | 2,4-dimethoxyphenyl                              |
| 49                     | do                                               | o-Chlorophenyl                                   | o-Chlorophenyl                                   |
| 50                     | do                                               | 2,4-dimethoxyphenyl                              | 2,4-dimethoxyphenyl                              |
| 51                     | do                                               | o-Methoxyphenyl                                  | o-Methoxyphenyl                                  |
| 52                     | do                                               | p-Methoxyphenyl                                  | p-Methoxyphenyl                                  |
| 53                     | do                                               | m-Phenylthio                                     | m-Phenylthio                                     |
| 54                     | o-Dimethylaminophenyl                            | o-Dimethylaminophenyl                            | o-Dimethylaminophenyl                            |
| 55                     | do                                               | p-Dipentylaminophenyl                            | p-Dipentylaminophenyl                            |
| 56                     | do                                               | o-Dipropylsulfamylphenyl                         | o-Dipropylsulfamylphenyl                         |
| 57                     | o-Dimethylcarbamylphenyl                         | o-Dimethylcarbamylphenyl                         | o-Dimethylcarbamylphenyl                         |
| 58                     | 2,4-dinaphthylthiophenyl                         | 2,4-dinaphthylthiophenyl                         | 2,4-dinaphthylthiophenyl                         |
| 59                     | 2,4-dipentylphenyl                               | 2,4-dipentylphenyl                               | 2,4-dipentylphenyl                               |
| 60                     | do                                               | 3,4-benzo(2-naphthyl)phenyl                      | 3,4-benzo(2-naphthyl)phenyl                      |
| 61                     | o-Dipentylaminophenyl                            | o-Dipentylaminophenyl                            | o-Dipentylaminophenyl                            |
| 62                     | 2,4-dipropoxyphenyl                              | 2,4-dipropoxyphenyl                              | 2,4-dipropoxyphenyl                              |
| 63                     | do                                               | o-Diethylcarbamylphenyl                          | o-Diethylcarbamylphenyl                          |
| 64                     | o-Dipropylcarbamylphenyl                         | o-Dipropylcarbamylphenyl                         | o-Dipropylcarbamylphenyl                         |
| 65                     | o-Ethoxyphenyl                                   | o-Ethoxyphenyl                                   | o-Ethoxyphenyl                                   |



wherein R<sub>1</sub> to R<sub>10</sub> are alkyl groups, e.g. lower alkyl groups of 1 to 6 carbon atoms; alkoxy groups, e.g. alkoxy groups containing 1 to 6 carbon atoms; chlorine, bromine or fluorine atoms; or substituents on adjacent carbon atoms in the phenyl ring together forming a benzo ring, e.g. an unsubstituted ring; with the proviso that at least one of the ortho positions in each of the phenyl groups B and D is unsubstituted. The dotted line circle stands for 4 delocalized electrons.

25 Representatives of the bi-imidazolyl compounds suited for being used according to the present invention are listed hereinafter in Table I.

TABLE I—Continued

| Number of the compound | R <sub>1</sub>               | R <sub>2</sub>                | R <sub>3</sub>                |
|------------------------|------------------------------|-------------------------------|-------------------------------|
| 66                     | o-Ethoxycarbonylphenyl       | o-Ethoxycarbonylphenyl        | o-Ethoxycarbonylphenyl        |
| 67                     | o-Ethylphenyl                | o-Ethylphenyl                 | o-Ethylphenyl                 |
| 68                     | o-N-ethylbutyramido-phenyl   | o-N-ethylbutyramido-phenyl    | o-N-ethylbutyramido-phenyl    |
| 69                     | o-N-ethylpropylaminophenyl   | o-N-ethylpropylaminophenyl    | o-N-ethylpropylaminophenyl    |
| 70                     | o-Ethylthiophenyl            | o-Ethylthiophenyl             | o-Ethylthiophenyl             |
| 71                     | o-N-ethylvaleramido-phenyl   | p-tert. Pentylophenyl         | p-tert. Pentylophenyl         |
| 72                     | o-Fluorophenyl               | o-Fluorophenyl                | o-Fluorophenyl                |
| 73                     | do                           | o-Methoxyphenyl               | o-Methoxyphenyl               |
| 74                     | o-Methoxyphenyl              | do                            | Do                            |
| 75                     | do                           | p-Chlorophenyl                | p-Chlorophenyl                |
| 76                     | do                           | p-Methoxyphenyl               | p-Methoxyphenyl               |
| 77                     | do                           | o-Methoxyphenyl               | o-Methoxyphenyl               |
| 78                     | do                           | p-Methoxyphenyl               | p-Methoxyphenyl               |
| 79                     | do                           | o-Methylthiophenyl            | o-Methylthiophenyl            |
| 80                     | do                           | p-Nitrophenyl                 | p-Nitrophenyl                 |
| 81                     | do                           | p-Phenylsulphonylphenyl       | p-Phenylsulphonylphenyl       |
| 82                     | o-Methoxycarbonylphenyl      | o-Methoxycarbonylphenyl       | o-Methoxycarbonylphenyl       |
| 83                     | do                           | 3,4-benzenophenyl             | 3,4-benzenophenyl             |
| 84                     | o-Methoxycarbonylphenyl      | p-N-ethylphenylsulphamyl      | p-N-ethylphenylsulphamyl      |
| 85                     | 2-methoxy-4-phenyl           | 2-methoxy-4-phenyl            | 2-methoxy-4-phenyl            |
| 86                     | o-Methylphenyl               | o-Methylphenyl                | o-Methylphenyl                |
| 87                     | do                           | p-Benzoyloxyphenyl            | p-Benzoyloxyphenyl            |
| 88                     | o-N-methylacetamido-phenyl   | o-N-ethylbutyramidophenyl     | o-N-ethylbutyramidophenyl     |
| 89                     | do                           | o-N-methylacetamidophenyl     | o-N-methylacetamidophenyl     |
| 90                     | o-N-methylpropionamidophenyl | o-N-methylpropionamidophenyl  | o-N-methylpropionamidophenyl  |
| 91                     | o-Methylthiophenyl           | o-Methylthiophenyl            | o-Methylthiophenyl            |
| 92                     | o-1-naphthylphenyl           | o-Phenoxyphenyl               | o-Phenoxyphenyl               |
| 93                     | o-2-naphthylphenyl           | o-2-naphthylphenyl            | o-2-naphthylphenyl            |
| 94                     | o-tert. Pentylophenyl        | o-tert. Pentylophenyl         | o-tert. Pentylophenyl         |
| 95                     | o-Pentyloxyphenyl            | o-Pentyloxyphenyl             | o-Pentyloxyphenyl             |
| 96                     | o-Pentyloxy carbonylphenyl   | o-Pentyloxy carbonylphenyl    | o-Pentyloxy carbonylphenyl    |
| 97                     | do                           | 3,4-benzenophenyl             | 3,4-benzenophenyl             |
| 98                     | o-9-phenanthrylphenyl        | p-Methoxyphenyl               | p-Methoxyphenyl               |
| 99                     | o-Phenoxyphenyl              | o-Phenoxyphenyl               | o-Phenoxyphenyl               |
| 100                    | do                           | 3,4,5-trimethoxyphenyl        | 3,4,5-trimethoxyphenyl        |
| 101                    | o-Phenyl(2-biphenyl)         | o-Phenyl(2-biphenyl)          | o-Phenyl(2-biphenyl)          |
| 102                    | o-Phenyl                     | p-Methoxycarbonylphenyl       | p-Methoxycarbonylphenyl       |
| 103                    | do                           | m-Pentyloxy carbonylphenyl    | m-Pentyloxy carbonylphenyl    |
| 104                    | do                           | p-Pentyloxy carbonylphenyl    | Do                            |
| 105                    | do                           | p-Phenyl                      | p-Phenyl                      |
| 106                    | o-Phenyliothio               | p-1-naphthylthiophenyl        | p-1-naphthylthiophenyl        |
| 107                    | o-Propoxyphenyl              | o-Propoxyphenyl               | o-Propoxyphenyl               |
| 108                    | 2,4,6-tribromophenyl         | 2,4,6-tribromophenyl          | 2,4,6-tribromophenyl          |
| 109                    | 2,4,6-triethylphenyl         | 2,4,6-triethylphenyl          | 2,4,6-triethylphenyl          |
| 110                    | 2,3,5-trichlorophenyl        | 2,3,5-trichlorophenyl         | 2,3,5-trichlorophenyl         |
| 111                    | 2,4,6-trichlorophenyl        | 2,4,6-trichlorophenyl         | 2,4,6-trichlorophenyl         |
| 112                    | do                           | o-Butylthiophenyl             | o-Butylthiophenyl             |
| 113                    | 2,4,6-tricyanophenyl         | p-Cyanophenyl                 | p-Cyanophenyl                 |
| 114                    | 2,4,6-triethoxyphenyl        | 2,4,6-triethoxyphenyl         | 2,4,6-triethoxyphenyl         |
| 115                    | 2,4,6-trimethoxyphenyl       | 2,4,6-trimethoxyphenyl        | 2,4,6-trimethoxyphenyl        |
| 116                    | 2,4,6-tri-tert. pentylphenyl | 2,4,6-tert-tert. pentylphenyl | 2,4,6-tert-tert. pentylphenyl |
| 117                    | 2,4,6-triisopropoxyphenyl    | 2,4,6-triisopropoxyphenyl     | 2,4,6-triisopropoxyphenyl     |
| 118                    | p-Chlorophenyl               | Phenyl                        | Phenyl                        |
| 119                    | p-Fluorophenyl               | do                            | Do                            |
| 120                    | Phenyl                       | p-Methoxyphenyl               | p-Methoxyphenyl               |
| 121                    | 3,4-dimethoxyphenyl          | Phenyl                        | Phenyl                        |
| 122                    | 5-acenaphthylphenyl          | do                            | Do                            |
| 123                    | 4-dimethylaminophenyl        | do                            | Do                            |
| 124                    | 3-nitrophenyl                | do                            | Do                            |
| 125                    | Phenyl                       | do                            | Do                            |

The last 8 compounds are C—C isomers. C—N isomers not listed in the Table I above and that are suited for being used according to the present invention have for R<sub>2</sub> and R<sub>3</sub> a phenyl group and for R<sub>1</sub> a 4-chlorophenyl or 4-fluorophenyl group.

The bi-imidazolyl compounds can be prepared according to methods described by Hayashi, C. S. in Bull. Chem. Soc., Japan, 33, 565 (1960), the French patent specification 1,351,818, filed Mar. 20, 1963 by Du Pont de Nemours, and the British patent specification 997,396, filed Mar. 21, 1963 by Du Pont de Nemours.

According to the preferably applied method the oxidative dimerisation is carried out in alkaline organic medium by means of a cyanoferrate(III) such as potassium cyanoferrate(III). According to that method normally a 1,2'-bi-imidazole (the C—N isomer) is obtained but sometimes also the 1,1'-, the 1,4'-, 2,2'-, 2,4'- and 4,4'-bi-imidazoles (the latter being the C—C isomer) mixed with the 1,2'-isomer.

For the purpose of the present invention it does not matter, however, which kind of isomer is used, as long as it effects the desired photo-oxidation of the reducing substance contained in the intermediate sheet.

Reducing compounds that—when intimately mixed with the bi-imidazolyl compounds—are capable to become oxidized by means of the photo-exposed bi-imidazolyl compounds belong to the class of organic compounds containing a Zerewitinoff hydrogen atom and more particularly, e.g., belong to one of the following classes:

(1) aromatic polyhydroxyl compounds and oxidizable derivatives, e.g. aromatic polyhydroxyl compounds wherein one of the hydroxyl groups has been substituted with an alkoxy group.

(2) aromatic polyamino compounds and their oxidizable derivatives, e.g. N-alkyl-substituted derivatives.

(3) aromatic hydroxylamino compounds and oxidizable derivatives thereof.

(4) compounds according to the following general formula:



wherein:

X represents oxygen, sulphur, —NH—, —CH<sub>2</sub>—, —CH=CH—, or



and

Z<sub>1</sub> and Z<sub>2</sub> each represent the necessary atoms to close a carbocyclic aromatic ring e.g. benzene ring including a substituted benzene ring.

Reducing compounds of class (1) are e.g.:

(1)





Reducing compounds of class (2) are e.g.:



Reducing compounds of class (3) are e.g.:



- Reducing compounds of class (4) are e.g.:
- (a) amino-9,10-dihydroacridines e.g. 3,6-bis(benzylamino)-9,10-dihydro-9-methyl-acridine, 3,6-bis(diethylamino)-9-hexyl-9,10-dihydro-acridine, 3,6-bis(diethylamino)-9,10-dihydro-9-methyl-acridine, 3,6-bis(diethylamino)-9,10-dihydro-9-phenyl-acridine, 3,6-diamino-9-hexyl-9,10-dihydroacridine, 3,6-diamino-9,10-dihydro-9-methylacridine, 3,6-diamino-9,10-dihydro-9-phenylacridine, 3,6-bis(dimethylamino)-9-hexyl-9,10-dihydro-acridine, and 3,6-bis(dimethylamino)-9,10-dihydro-9-methyl-acridine.
  - (b) aminodihydrophenazines e.g. 3,7-bis(benzylethylamino)-5,10-dihydro-5-phenyl-phenazine, 3,7-bis(diethylamino)-5-hexyl-5,10-dihydro-phenazine, 3,7-bis(dihexylamino)-5,10-dihydrophenazine, 3,7-bis(dimethylamino)-5-(p-chlorophenyl)-5,10-dihydrophenazine, 3,7-diamino-5-(o-chlorophenyl)-5,10-dihydro-phenazine, 3,7-diamino-5,10-dihydrophenazine, 3,7-diamino-5,10-dihydro-5-methylphenazine, 3,7-diamino-5-hexyl-5,10-dihydrophenazine, 3,7-bis(dimethylamino)-5,10-dihydrophenazine, 3,7-bis(dimethylamino)-5,10-dihydro-5-phenyl-phenazine, and 3,7-bis(dimethylamino)-5,10-dihydro-5-methyl-phenazine.
  - (c) aminophenothiazines e.g. 3,7-bis(dimethylamino)-phenothiazine, 3,7-bis(dimethylamino)-4,6-dimethylpheno-thiazine, 3,7-bis(diethylamino)-2,8-dimethylphenothiazine, 3,7-bis(dimethylamino)-4-nitrophenothiazine, 3,7-bis(dibutylamino)-phenothiazine, 3-diethylamino-7-dimethylaminophenothiazine, 3-dimethylamino-7-N-benzyl-N-methylamino-phenothiazine, and 3,7-bis(N-benzyl-N-ethylamino)-phenothiazine.
  - (d) aminophenoxazines e.g. 3,7-bis(dimethylamino)-phenoxazine, 3,7-bis(diethylamino)-phenoxazine, 3,7-bis(dibutylamino)-phenoxazine, 3-diethylamino-7-dimethylamino-2-methyl-phenoxazine, 3-dimethylamino-7-dipropylaminophenoxyazine, 5-dimethylamino-9-diethylamino-12H-benzo[a]phenoxazine, 5-dibenzylamino-9-diethylamino-12H-benzo[a]phenoxazine, and 5,9-bis(diethylamino)-12H-benzo[a]phenoxazine.

Preferably used oxidizable compounds are volatilizable e.g. between a temperature of 60 to 140° C.

The light-sensitive sheets used according to the present invention contain at least one biimidazolyl compound in a ratio from 2 to 5 mole to 1 mole of reducing agent. Preferably the biimidazolyl compound is applied in an amount of 0.5 to 2 g. per sq.m., but the amount can be adapted according to the requirements of the copying process and the kind of reductor and reducible substance.

For the preparation of the above described intermediate sheet the biimidazolyl compound and reducing agent which is transferable by heat in volatilized or molten state, are applied together from a solution or dispersion preferably in the presence of a film-forming binding agent.

As binding agent for the photosensitive layer all kinds of natural, modified natural and synthetic resins can be used, e.g. proteins such as gelatine, cellulose derivatives, e.g. a cellulose ether such as ethylcellulose, cellulose esters, carboxymethylcellulose, alginic acid and derivatives, starch ethers, galactomannan, polyvinyl alcohol, poly-N-vinylpyrrolidone, polymers derived from  $\alpha,\beta$ -ethylenically unsaturated compounds, e.g. homo- and co-vinyl polymers such as polyvinyl chloride, copolymers of vinyl chloride and vinyl acetate partially saponified polyvinylacetate, copolymers of acrylonitrile and acrylamide, polyacrylic acid esters, polymethacrylic acid esters, or polyethylene.

The photosensitive material may consist of a self-supporting sheet by using a film-forming binding agent to attain that result, or may comprise a photosensitive layer applied to a support. Suitable supports are, e.g., paper supports of which glassine paper is a preferred one, and resin supports known in silver halide photography. It is also possible to apply the photosensitive material to glass or metal plate or to a support from which it can be stripped off and transferred to a permanent support.

A receptor material used in conjunction with the photosensitive material contains a substance that is a reactive component in a colour reaction with the reducing compound contained in the photosensitive sheet.

Such substances belong to a wide diversified group of chemicals so that it is practically impossible to characterize them by a particular chemical structure.

A practical test that can be used to know whether a particular reducible compound used in a receiving sheet is suited or not to produce a visible colour change is to heat the elected reaction partners in one of the above binding agents or an inert solvent beyond a temperature of 60° C. with a particular reaction partner to be used in the receiving sheet, and to take notice, e.g. between 80 and 120° C. of the degree of colour change in the layer or test tube.

A relatively high reactivity of a particular reducing agent with the photoexposed biimidazolyl compound is important to obtain clear copies on the receptor sheet within a suitable exposure and processing time.

Here again a practical test will make it possible to choose a proper combination of reducing agent and biimidazolyl compound that gives an optimal result.

Reaction partners for at least some of the reducing compounds of the classes (1) to (4) forming a coloured product therewith are listed in the following Groups (I), (II), (III) and (IV).

(I) Heavy metal compounds especially of metals of the third, fourth and fifth main group as well as of the I<sup>st</sup>, the II<sup>nd</sup>, the VI<sup>th</sup>, the VII<sup>th</sup> and the VIII<sup>th</sup> auxiliary group of the Periodic Table, e.g. compounds of the following heavy metals: cadmium, mercury, iron, cobalt, nickel, copper, silver, gold, bismuth and thallium. Especially suitable are salts of these metals with long chained aliphatic carboxylic acids, e.g. nickel stearate, cobalt palmitate, iron stearate, the addition compound of bismuth nitrate with an amine, e.g. triethanolamine. Particularly suited are noble metal compounds e.g. silver compounds, which under the conditions of the copying process of the present invention are extremely non-light-sensitive, e.g. the silver salts of aliphatic carboxylic acids with a thioether group such as those described e.g. in the British patent specification 1,111,492 filed Aug. 13, 1965 by Agfa A.G., or silver salts of long-chained aliphatic (preferably at least C<sub>14</sub>) carboxylic acids such as silver behenate, silver palmitate, silver stearate and others.

On applying the above mentioned heavy metal compounds in general brown to black copies are obtained. The image consists of the metal in question and/or of a reaction product of the transferred image forming compound.

## 11

(II) Colour couplers with which the transferred reducing compounds by oxidative coupling react image-wise to dyestuffs, (e.g. suitable couplers for arylamines are described in the United Kingdom patent specification 1,160,224, filed Dec. 14, 1965 by Gevaert-Agfa N.V.).

(III) Diazonium salts for coupling with phenols or naphthols that contain e.g. an amino group, so that coloured compounds are formed as are known from diazotype recording.

(IV) Leucophthalocyanine: As far as leucophthalocyanines were not prepared from ready phthalocyanines, or could not be synthesized therefrom, they are also designated as phthalocyanine preproducts. This term has been employed e.g. in the article of B. R. A. Brooks, J. G. Burt, B. F. Skiles and M. S. Whelen, *J. Org. Chem.*, 24, 383 (1959). In the related chapter of Ullmanns Encyklopädie der Technischen Chemie, 34th edition, vol. 13 the term "phthalocyanine metal complexes" has been used for the same types of substances for which in connection with the present invention the term "leucophthalocyanines" has been used. The latter term is explained e.g. in the U.S. patent specification 2,772,285 of Robert A. Brooks, issued Nov. 27, 1956. In this specification it relates only to leuco copper phthalocyanine, but also applies to the corresponding complexes with other phthalocyanine-binding metal. According to this specification leucophthalocyanines are colourless or but light coloured products, in which the phthalocyanine frame already is developed completely, and that can be converted to phthalocyanines by a reduction process. In this reduction process constituents can be split off occasionally simultaneously, which constituents are comprised by the molecule of the leucophthalocyanine and not by the phthalocyanine. The preparation of such leucophthalocyanine can occur e.g. if first of all a phthalocyanine, e.g. a metal free phthalocyanine or CuPc (Pc=phthalocyanine), NiPc, CoPc or ZnPc are prepared, and thereupon are provided of additional ligands under oxidative conditions, or if a reaction mixture which is suited in itself for the preparation of the phthalocyanine, is heated below the temperature required therefore is reached, or if the reduction potential necessary for the formation of the phthalocyanine is not applied.

Especially suited are metal containing leucophthalocyanines for the metal free leucophthalocyanines are relatively instable. Especially favourable are the very stable and little coloured leuco-cobalt-phthalocyanines.

To be mentioned especially are leuco-cobalt-phthalocyanines described e.g. in *Zeitschrift für Angewandte Chemie*, 68, 145 (1956), such as e.g. the phthalocyanine-cobalt-ethylenediamine complex. Instead of ethylene diamine other diamines or polyamines can be built in as ligands, such as

propylenediamine-(1,2) and propylenediamine-(1,3), mono-ethylpropylenediamine-(1,3), hydroxyethyl-ethylenediamine, N-methyl-N-β-hydroxyethylpropylenediamine, N,N'-diethyl-ethylenediamine, N,N-di-(β-aminoethyl)-ethylenediamine, N,N'-di(β-aminoethyl)-ethylenediamine, N,N'-di[β-(β-aminoethyl)-aminoethyl]-amine or

also monoamines such as 3-(2-ethylhexyloxy)-propylamine(1) or stearylamine. The solubility properties of the corresponding leuco-cobalt phthalocyanine depend on the nature of the built in amine.

According to another embodiment of the method according to the present invention a partner for a colour forming reaction in the receiving layer is absolutely superfluous. This applies for the image-forming phenols or naphthols, which on heating with themselves or in the

## 12

presence of aerial oxygen yield sufficiently coloured compounds. In this case simple uncoated paper stock can be used as receiving material.

In addition to the actual image-forming reaction partners the image-receiving layers may contain further additives which ameliorate the colour tone e.g. 1-(2H)-phthalazinone, as toner, and which accelerate the reaction for the formation of the image substance, e.g. sterically hindered phenols that on heating become reactive partners in the reduction reaction e.g. 2,4,6-tri-tert.butylphenol. Suitable image-receiving layers are known already e.g. from the U.S. patent specifications 3,094,417 of Wesley R. Workmans, issued June 18, 1968, 3,094,619 of Edwin A. Grant, Jr., issued June 18, 1963 and 3,094,620 of John L. Reitter, issued June 18, 1963 and in the German patent specifications 895,101 filed Nov. 10, 1944 by I. G. Farbenindustrie; 1,003,577, filed Feb. 11, 1955 by Agfa A.G.; 1,159,758, filed Sept. 9, 1962 by Agfa A.G.; 1,004,043, filed Feb. 7, 1955 by Agfa A.G. and 1,165,410, filed Sept. 15, 1962 by Agfa A.G., the Dutch patent specification 277,086 filed Apr. 11, 1962 by Gevaert Photo-Producten N.V. and the Belgian patent specifications 614,064, filed Aug. 20, 1962 by Gevaert Photo-Producten N.V. and 609,057, filed Apr. 12, 1962 by Gevaert Photo-Producten N.V.

For the exposure of the light-sensitive layers according to this invention the usual light source for copying purposes can be used here e.g. mercury lamps, iodine quartz lamps or incandescent lamps. The inherent spectral sensitivity of the photo-sensitive materials depends on the nature of the biimidazolyl compounds used. Most biimidazolyl compounds are sensitive to ultraviolet light of a wavelength below 300 nm. The spectral sensitizability of said compounds makes it possible, however, to use visible light for the exposure step.

A direct exposure as well as a contact reflex exposure can be applied, reflex exposure being particularly interesting for the reproduction of graphic originals having light-absorptive image areas on an opaque reflecting background.

Transfer of image forming compounds from the unexposed areas of the light-sensitive layers in the image-receiving layer occurs preferably at a temperature, comprised between 80 and 200°C. Heating can occur e.g. by conveying the exposed light-sensitive layer in contact with an image-receiving layer over hot plates or rollers or by irradiation with infrared light. The most favourable temperature and time of heating of course depends on the nature of the image-forming compound to be formed and can be obtained by few simple tests.

As spectral sensitizing agent for the photosensitive material according to this invention practically a number of compounds are suited, which also have been used for the spectral sensitization of silver halide emulsion layers. These are preferably cyanine dyes, merocyanines, styryl dyes and rhodacyanine of all sorts, e.g. as described by F. M. Hamer, *The Cyanine Dyes and related Compounds*, 1964, e.g. as described on pages 90, 100, 433, 502 and 511.

In this respect methine dyes according to the three following general Formulae A, B or C are preferably used.



wherein:

each of Z and Z' represents an oxygen atom or a N—R<sub>1</sub> group wherein R<sub>1</sub> represents an alkyl group or a sub-

## 13

substituted alkyl group, e.g. a C<sub>1</sub>-C<sub>4</sub> alkyl group such as methyl, ethyl, n-propyl, n-butyl, benzyl, phenylethyl, a cycloaliphatic group, an unsaturated aliphatic group, e.g. allyl, or an aryl group e.g. a mononuclear aromatic group of the benzene series, such as phenyl, or o-, m- or p-tolyl,

R<sub>3</sub> represents hydrogen or a lower alkyl group e.g. methyl or ethyl,

each of R<sub>2</sub> and R<sub>4</sub> represents a substituent of the type contained in cyanine dyes on the cyanine nitrogen atom, e.g. an alkyl group such as methyl, ethyl, propyl, isopropyl, butyl, isobutyl including a substituted alkyl group such as  $\beta$ -hydroxyethyl,  $\beta$ -acetoxyethyl, carboxymethyl and carboxyethyl as described in the German patent specification 704,141, filed Mar. 9, 1938 by I. G.

Farbenindustrie A.G., sulphaalkyl as described in the United Kingdom patent specification 742,112, filed Oct. 23, 1952 by Agfa (Farbenfabriken Bayer), such as sulphoethyl, sulphopropyl, sulphobutyl, sulphatoalkyl as described in the French patent specification 1,149,769, filed May 14, 1956 by Veb Filmfabrik Agfa Wolfen, such as sulphatopropyl and sulphatobutyl, the group —A—CO—O—B—SO<sub>2</sub>—OH wherein A and B have the same significance as set forth in United Kingdom patent specification 886,271, filed June 20, 1957 by Gevaert Photo-Producten N.V. such as a sulphocarbomethoxymethyl group, a  $\omega$ -sulphocarbopropoxymethyl group, a  $\omega$ -sulphocarbobutoxymethyl group, a p-( $\omega$ -sulphocarbobutoxy)-benzyl group, the group —A—W—NH—V—B wherein A, W, V and B have the same significance as set forth in United Kingdom patent specification 904,332, filed July 5, 1957 by Gevaert Photo-Producten N.V. such as a N-(methylsulphonyl)-carbamyl-methyl group,  $\gamma$ -(acetylsulphamyl)-propyl, a  $\delta$ -(acetylsulphamyl)-butyl group, the group



wherein A has the same significance as described in the United Kingdom patent specification 886,270, filed June 24, 1957 by Gevaert Photo-Producten N.V., an aralkyl group such as a benzyl group or a substituted aralkyl group such as carboxybenzyl and sulphobenzyl, an aryl group such as phenyl or a substituted aryl group such as carboxyphenyl, a cycloalkyl group such as cyclohexyl or an allyl group,

each of Y and Y' represents a substituent having an electronegative character e.g. halogen such as chlorine, bromine or fluorine, a cyano group, an acyl group e.g. acetyl group, a carbamyl group or a substituted carbamyl group e.g. a R<sub>1</sub>—NHCO— group, wherein R<sub>1</sub> is a group identical to R<sub>1</sub> above, a sulphamyl group, or a substituted sulphamyl group, e.g. a



group wherein R<sub>1</sub> has the same significance as described above,

m is a positive integer 1, 2 or 3,

n is a positive integer indicating the number of substituents on the benzene nucleus, and

X<sup>-</sup> is an anion e.g. Cl<sup>-</sup>, Br<sup>-</sup>, I<sup>-</sup>, ClO<sub>4</sub><sup>-</sup>, CH<sub>3</sub>SO<sub>4</sub><sup>-</sup> or



but is not present when the R<sub>2</sub> group contains already an anionic part (betaine-structure) e.g. —SO<sub>3</sub><sup>(-)</sup>, —OSO<sub>3</sub><sup>(-)</sup>, —COO<sup>(-)</sup>,

## 14



wherein:

R<sub>1</sub> represents an alkyl group or a substituted alkyl group e.g. a C<sub>1</sub>-C<sub>4</sub> alkyl group, such as methyl, ethyl, n-propyl, n-butyl, benzyl, phenylethyl, a cycloaliphatic group, an unsaturated aliphatic group, e.g. allyl, or an aryl group e.g. a mononuclear aromatic group of the benzene series such as phenyl, or o-, m- or p-tolyl, each of L<sub>1</sub>, L<sub>2</sub>, L<sub>3</sub> and L<sub>4</sub> represents a methine group, or a substituted methine group, e.g. a methine group substituted with a lower alkyl group,

Z represents the atoms necessary to complete a heterocyclic nitrogen-containing nucleus comprising 5 to 6 atoms in the heterocyclic ring such as those of the thiazole series (e.g. thiazole, 4-methylthiazole, 4-phenylthiazole, 5-methylthiazole, 5-phenylthiazole, 4,5-dimethylthiazole, 4,5-diphenylthiazole, 4-(2-thienyl)-thiazole), those of the benzothiazole series (e.g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, 4,5,6,7-tetrahydrobenzothiazole, 5,6-dimethoxybenzothiazole, 5,6-dioxymethylenebenzothiazole, 5-hydroxybenzothiazole, 6-hydroxybenzothiazole, 5,6-dimethylbenzothiazole), those of the naphthothiazole series (e.g. naphtho[2,1-d]thiazole, naphtho[1,2-d]thiazole, 5-methoxynaphtho[1,2-d]thiazole, 5-ethoxynaphtho[1,2-d]thiazole, 8-methoxynaphtho[2,1-d]thiazole, 7-methoxynaphtho[2,1-d]thiazole), those of the thianaphtho[7,6-d]thiazole series (e.g. 7-methoxythianaphtho[7,6-d]thiazole), those of the oxazole series (e.g. 4-methyloxazole, 5-methyloxazole, 4-phenyloxazole, 4,5-diphenyloxazole, 4-ethyloxazole, 4,5-dimethyloxazole, 5-phenyloxazole), those of the benzoxazole series (e.g. benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 6-methoxybenzoxazole, 5-hydroxybenzoxazole, 6-hydroxybenzoxazole), those of the naphthoxazole series (e.g. naphtho[2,1-d]oxazole, naphtho[1,2-d]oxazole), those of the selenazole series (e.g. 4-methylselenazole, 4-phenylselenazole), those of the benzoselenazole series (e.g. benzoselenazole, 5-chlorobenzoselenazole, 5-methoxybenzoselenazole, 5-hydroxybenzoselenazole, 4,5,6,7-tetrahydrobenzoselenazole), those of the naphthoselenazole series (e.g. naphtho[2,1-d]selenazole, naphtho[1,2-d]selenazole), those of the thiazoline series (e.g. thiazoline, 4-methylthiazoline, 4-hydroxymethyl-4-methylthiazoline, 4,4-bis-hydroxymethylthiazoline, 4-acetoxyethyl-4-methylthiazoline, 4,4-bis-acetoxyethylthiazoline), those of the oxazine series (e.g. oxazoline, 4-hydroxymethyl-4-methyloxazoline, 4,4-bis-hydroxymethyl-oxazoline, 4-acetoxyethyl-4-methyloxazoline, 4,4-bis-acetoxyethyl-oxazoline), those of the selenazoline

series (e.g. selenazoline), those of the 2-quinoline series (e.g. the quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline), those of the 4-quinoline series (e.g. quinoline, 6-methoxyquinoline, 7-methylquinoline, 8-methylquinoline), those of the pyrrolidine series (e.g. 1-ethyl-pyrrolidine or 1-methyl-pyrrolidine, those of the 3,3-dialkylindolenine series (e.g. 3,3 - dimethylindolenine, 3,3,5 - trimethylindolenine, 3,3,7 - trimethylindolenine), those of the pyridine series (e.g. pyridine, 5-methylpyridine), those of the benzimidazole series (e.g. 1-ethylbenzimidazole, 1-phenylbenzimidazole, 1-ethyl-5-chloro - 6 - bromobenzimidazole, 1-ethyl-5-phenylbenzimidazole, 1-ethyl-5-fluorobenzimidazole, 1-ethyl-5,6-difluorobenzimidazole, 1 - ethyl-5-cyanobenzimidazole, 1-( $\beta$ -acetoxethyl) - 5 - cyanobenzimidazole, 1-ethyl-5-chloro-6-cyanobenzimidazole, 1-ethyl-5-fluoro-6-cyanobenzimidazole, 1-ethyl-5-acetylbenzimidazole, 1-ethyl-5-chloro-6-fluorobenzimidazole, 1-ethyl-7-carboxybenzimidazole, 1-ethyl-7-carboxybenzimidazole, 1-ethyl-5-carbethoxybenzimidazole, 1-ethyl - 7 - carbethoxybenzimidazole, 1-ethyl - 5 - sulphamylbenzimidazole, or 1-ethyl-5-N-ethyl-sulphamylbenzimidazole,

*n* represents 1 or 2,

*m* represents 2 or 3, and

each of P and Q represents an electronegative substituent, or

P and Q together represent the necessary atoms to close a cyclic ketomethylene nucleus e.g. an imidazolone-thione or rhodanine nucleus.



wherein:

each of R'<sub>1</sub> and R'<sub>2</sub> represents an alkyl group, e.g. a (C<sub>1</sub>-C<sub>4</sub>) alkyl group or an aralkyl group, e.g. a benzyl group, each of L<sub>1</sub>, L<sub>2</sub>, L<sub>3</sub> and L<sub>4</sub> represents a methine group, including a substituted methine group, Ar represents a bivalent aromatic nucleus, e.g. a phenylene group,

*p* represents 1 or 2,

*q* represents 2 or 3, and

Z represents the atoms necessary to complete a heterocyclic nitrogen containing nucleus comprising 5 to 6 atoms in the heterocyclic ring e.g. a pyridine nucleus, a thiazole nucleus, an oxazoline or a quinoline nucleus.

The sensitizing agents may be added to the photosensitive composition in a suitable solvent such as short chained aliphatic alcohols or aqueous systems. The concentration of the spectral sensitizing agent(s) may vary within wide limits. In general amounts comprised between 0.05 and 0.3 mole/per mole of biimidazolyl compound have been proved as sufficient.

The most suitable sensitizing agents for a particular biimidazolyl compound can be determined by means of the usual sensitometric tests, without difficulty by those skilled in the art.

By the addition of sensitizing agents not only an increase of sensitivity is reached but also a marked increase of the general sensitivity, which is desirable for obtaining shorter times of copying. By the possibility of sensitization of layers according to this invention also for the red and green region of the spectrum it is possible not only to copy coloured originals in an unobjectional way but also to prepare copies in natural colours by a suitable choice of the image forming systems which yield dye-stuffs in the subtractive selection colours.

In order to obtain stable positive direct legible copies of graphic originals having differentially light-absorptive image and background areas the photo-oxidizing biimidazolyl compound is preferably used in combination with a volatilizable reducing agent in a sheet, which is the so-called intermediate sheet, a preferred reducing agent for that purpose is 4-methoxynaphthalol.

Said sheet co-operates after its information-wise electromagnetic irradiation with a receiving material, the so-called receptor sheet that contains a reducible substance, e.g. silver behenate, for producing a colour reaction with the reducing agent transferred by heat after the information-wise exposure of the intermediate sheet.

It is possible to obtain copies of transparent as well as of opaque originals in a unitary photothermosensitive copy sheet by using e.g. on a thin transparent paper-like backing a thin coating comprising said reducible substance, kept out of direct chemical contact with respect to the reducing agent and the photo-oxidizing biimidazolyl compound by means of a thin non-transparent highly pigmented vapour-permeable binder layer the binding agent of which is not soluble in the solvent from which the photosensitive top-coat is applied.

The unitary photothermosensitive copy sheet yields when applied in a reflux exposure technique a copy that is directly legible through the rear side of the transparent support.

A pigment such as titanium dioxide and zinc oxide having an average grain size of 5 to 1 $\mu$  when applied in an ethyl cellulose binder allow the vaporized reducing agent e.g. 4-methoxynaphthalol to pass through the vapour permeable interlayer and to react with the reducible substance e.g. silver behenate.

The permeable layer may alternatively be replaced by a normally impermeable thin coating of a fusible film-forming material which melts and becomes compatible with the underlaying binder medium for the reducible substance. (See for such technique and suitable substances the United Kingdom patent specification 1,184,054, filed Apr. 5, 1966 by Gevaert-Agfa N.V. and the U.S. patent specification 3,223,838 of Shioichiro Hoshino and Akira Kato, issued Dec. 14, 1965.)

Heat may be applied by conventional thermographic front-printing procedures using infra-red radiation. Replacing the printed original with a continuously infrared-absorptive black paper, plate, roller and irradiating that absorptive material in contact with the photothermosensitive sheet causes overall reproducible heating.

It is of course possible to use other kinds of energy sources to produce heat, of which electrical resistance heating and high frequency current heating and induction heating are a few examples.

Instead of transferring the reducing agent in volatilized state it is possible to transfer it in a fusible medium, e.g. a fusible waxy or resinous medium. Transfer can be speeded up by using a solvent causing some swelling as described in the United Kingdom patent specification 1,135,371, filed Jan. 7, 1966 by Agfa-Gevaert A.G. Heat transfer of polymer substrata without solvent swelling is described e.g. in the Belgian patent specification 700,-472, filed June 26, 1967 by Gevaert-Agfa N.V. corresponding with the United Kingdom patent specification 1,195,842, filed June 24, 1966 by Gevaert-Agfa N.V.

The following examples illustrate the present invention. Parts are parts by weight unless otherwise indicated.

#### EXAMPLE 1

A photosensitive intermediate sheet was prepared by coating a glassine type paper base in a ratio of 40 g. per sq.m. with a solution of the following composition:

|                                                          |    |     |
|----------------------------------------------------------|----|-----|
| Bis[2 - (o - chlorophenyl) - 4,5 - diphenyl - imidazole] | g  | 10  |
| 4-methoxy-1-naphthol                                     | g  | 1   |
| Ethylcellulose                                           | g  | 10  |
| 2-butanone                                               | ml | 500 |

17

The resulting sheet was dried and irradiated for 12 sec. through a positive transparency of a printed text by means of an ultraviolet light source (1000 w.-lamp) placed at a distance of 5 cm. from the intermediate sheet.

Subsequently the irradiated sheet was pressed for 5 sec. with its photosensitive layer in contact at 125° C. with a receptor sheet, which is a white paper prepared by coating and drying thereon a continuous thin colourless layer of a ball-milled mixture of silver behenate, phthalazinone as toning agent, 2,6-di-tert.-butyl-4-methylphenol as heat-sensitive reductor, poly-tert.-butyl methacrylate as binding agent (3 parts for every 10 parts of silver behenate) and 86 parts of acetone. The dried receptor sheet contained per sq.m. an amount of silver behenate equivalent with 0.2 g. of silver per sq.m. 400 mg. per sq.m. of phthalazinone, and 40 mg. per sq.m. of 2,6-di-tert.-butyl-4-methylphenol.

A sharp, positive, black copy of the transparency was obtained.

## EXAMPLE 2

A photosensitive intermediate sheet was prepared by coating a map overlay tracing paper in a ratio of 50 g. per sq.m. with a solution of the following composition:

|                                                          |    |     |
|----------------------------------------------------------|----|-----|
| Bis[2 - (o - chlorophenyl) - 4,5 - diphenyl - imidazole] | g  | 10  |
| 2,5-di-tert.-butyl-hydroquinone                          | g  | 1   |
| Ethylcellulose                                           | g  | 10  |
| Chloroform                                               | ml | 500 |

After exposure for 15 sec. and transfer contact as described in Example 1 a sharp brown positive print of the original was obtained.

## EXAMPLE 3

A transparent subbed polyester film of 0.10 mm. thickness was supplied in a ratio of 30 g. per sq.m. with a solution of the following composition:

|                                                          |    |     |
|----------------------------------------------------------|----|-----|
| Bis[2 - (o - chlorophenyl) - 4,5 - diphenyl - imidazole] | g  | 10  |
| p-Phenylenediamine                                       | g  | 1   |
| Cellulose acetate butyrate (half second butyrate)        | g  | 10  |
| 2-butanone                                               | ml | 500 |

After image-wise exposure the dried coating was contacted for 5 sec. as described in Example 1 whilst heating at 120-130° C. with a receiving paper sheet the receptor layer of which was prepared from a solution as described hereinafter.

|                                                                                                                                |    |     |
|--------------------------------------------------------------------------------------------------------------------------------|----|-----|
| N-(2,4-dinitrophenyl)-pyridinium chloride                                                                                      | g  | 5   |
| Saponine                                                                                                                       | g  | 0.2 |
| Polyoxyethylene - hydroxyethylcellulose (marketed under the trade name "Cellosolve WP 09" by Union Carbide & Carbon, New York) | g  | 1   |
| Water                                                                                                                          | ml | 100 |

A dark-brown positive image on a yellow background was formed.

## EXAMPLE 4

The intermediate sheet of Example 1 was sensitized to visible light by adding to the coating composition for every 500 ml. 1 g. of 2-(p-dimethylaminostyryl)-benzothiazole as spectrally sensitizing agent.

A direct exposure for 30 sec. through a positive transparency with a tungsten filament light source of 1500 w. placed at a distance of 10 cm. from the intermediate sheet made it possible to produce a sharp positive black

18

copy on contact-heating transfer as described in Example 1.

By using as original a black printed text on an opaque white background a reflex exposure yielded after a 15 to 25 sec. irradiation with the same light source a brown positive print on the same receptor sheet.

## EXAMPLE 5

10 The photosensitive intermediate sheet of Example 3 was sensitized to visible light by adding to every 500 ml. of said solution 1 g. of a spectral sensitizing merocyanine dye containing a rhodanine nucleus and having the following structural formula:



## EXAMPLE 6

A solution suited for preparing an intermediate photosensitive sheet was prepared as follows:

20 g. of di(2,4,5-triphenylimidazole) were dissolved in 350 ml. of 2-butanone. The pink solution obtained discoloured after a few hours standing at room temperature, an isomerisation according to the following scheme had taken place:

35



19

## EXAMPLE 7

On tracing paper the following composition was coated in a ratio of 40 g./sq.m.:

|                                               |     |
|-----------------------------------------------|-----|
| Di[2-(o-chlorophenyl)-4,5-diphenyl-imidazole] | 15  |
| N,N-diethyl-p-phenylenediamine                | 1   |
| Ethylcellulose                                | 10  |
| 2-butanol                                     | 500 |

After an image-wise exposure with U.V. light for 10 seconds by means of a 1000 w. lamp, the layer was pressed at 120-130° C. for 5-7 seconds on a paper that had been impregnated with the following 2 compositions (A) and (B):

|                                       |     |
|---------------------------------------|-----|
| (A)                                   |     |
| Potassium persulphate                 | 2   |
| 1 N sodium hydroxide solution         | 5   |
| Saponine                              | 0.5 |
| Polyoxyethylene hydroxyethylcellulose | 0.5 |
| Water                                 | 45  |

After drying the following composition (B) was applied thereto.

(B) N-hexadecyl-1-hydroxy-4-chloro-2-naphthoic acid amide having the formula:



A material was obtained which was then exposed as described in Example 8. A positive, cyan copy was obtained.

## EXAMPLE 8

In order to obtain a yellow image on a receiving layer prepared as described in Example 7, the 2-naphthoic acid amide compound of composition (B) was replaced by 1 g. of benzoylacetanilide.

## EXAMPLE 9

By replacing in the receiving layer N-hexadecyl-1-hydroxy-4-chloro-2-naphthoic acid amide by 1 g. of p-nitrophenyl-methylsulphide a magenta image was obtained.

## EXAMPLE 10

If in the light-sensitive composition of Example 7 1 g. of 2-(4-dimethylamino-styryl)-quinoline was added for every 500 ml., exposure could be carried out with visible light (1500 watt lamp for 20-30 seconds) through a transparent original or to an opaque original.

## EXAMPLE 11

A U.V. light-sensitive layer was obtained by coating a polyester film or tracing paper with the following composition:

|                                                         |     |
|---------------------------------------------------------|-----|
| Di[2 - phenyl - 4,5 - di - (p-methoxyphenyl)-imidazole] | 20  |
| Phenothiazine                                           | 2   |
| Ethylcellulose                                          | 20  |
| 2-butanol                                               | 350 |

75

20

As a receiving layer a material comprising silver behenate can be used. A sharp, black, positive image was obtained.

## EXAMPLE 12

The material of Example 11 could be used by employing as a receiving layer a paper which had been coated with the following mixture that had been ball-milled for 10 hours:

|    |                                                                                                                          |     |
|----|--------------------------------------------------------------------------------------------------------------------------|-----|
| 5  | Mercury(II) stearate                                                                                                     | 2   |
| 10 | Copoly(vinylchloride vinyl acetate vinylalcohol)<br>(sold under the trade name Vinylite VAGH by<br>Bakelite Corporation) | 2   |
| 15 | 2-butanol                                                                                                                | 100 |

After exposure as described in Example 8 a brownish violet image was obtained.

## EXAMPLE 13

Example 11 was repeated but the phenothiazine in the photosensitive material was replaced by phenoxazine. After exposure as described in Example 8 a black image was obtained.

## EXAMPLE 14

Example 13 was repeated but mercury(II) stearate was incorporated into the receiving layer. After exposure as described in Example 6 a brown image was obtained.

## EXAMPLE 15

A photosensitive intermediate sheet was prepared by 35 coating a glassine type paper base in a ratio of 40 g. per sq.m. with a solution of the following composition:

|    |                                                          |     |
|----|----------------------------------------------------------|-----|
| 40 | Bis[2 - (o - chlorophenyl) - 4,5 - diphenyl - imidazole] | 10  |
| 45 | 4-methoxy-1-naphthol                                     | 1   |
| 45 | A sensitizing dye listed in the table herein-after       | 5   |
| 45 | Ethylcellulose                                           | 10  |
| 45 | 2-butanol                                                | 500 |

The resulting sheet was dried and irradiated for 2 min. through a step wedge having consecutive steps with optical density increments of 0.1.

In the exposure a visible light emitting light source 50 (1500 w.-incandescent halogen containing lamp) placed at a distance of 5 cm. from the intermediate sheet was used.

Subsequently to the irradiation the sheet was pressed at 120° C. for 5 sec. with its photosensitive layer in contact 55 with a receptor sheet which is a white paper prepared by coating and drying thereon a continuous thin colourless layer of a ball-milled mixture of silver behenate, phthalazinone as toning agent, 2,6-di-tert.-butyl-4-methylphenol as heat-sensitive reductor, poly-tert.-butyl methacrylate as binding agent (3 parts for every 10 parts of silver behenate) and 86 parts of acetone. The dried receptor sheet contained per sq.m. an amount of silver behenate equivalent with 0.2 g. of silver per sq.m., 400 mg. per sq.m. of phthalazinone, and 40 mg. per sq.m. of 2,6-di-tert.-butyl-4-methylphenol.

In each case a positive black wedge print was obtained. In the following Tables A, B and C the first wedge step that is visible reproduced on the receiving material is given for each differently sensitized photosensitive intermediate sheet. The higher that number, the higher the sensitivity since it indicates the amount of steps in the photosensitive intermediate sheet, in which the reducing 70 4-methoxy-1-naphthol has been transformed into a non-reducing state by means of the photo-exposed dye sensitized biimidazolyl compound.



| No. of test | (Y') <sub>n</sub>                   | R <sub>2</sub>                   | Z                             | (Y') <sub>n</sub>                                            | R <sub>4</sub>                  | Z'                               | R <sub>3</sub>    | X-                                            | m              | First visible step | Sens. max. (nm.) |     |
|-------------|-------------------------------------|----------------------------------|-------------------------------|--------------------------------------------------------------|---------------------------------|----------------------------------|-------------------|-----------------------------------------------|----------------|--------------------|------------------|-----|
| Blank       |                                     |                                  |                               |                                                              |                                 |                                  |                   |                                               |                |                    |                  |     |
| 1           | 6-Cl                                | C <sub>2</sub> H <sub>5</sub>    | N-CH <sub>3</sub>             | 6-Cl                                                         | C <sub>2</sub> H <sub>5</sub>   | N-CH <sub>3</sub>                | H                 | I <sup>-</sup>                                | 2              | 7                  | 507              |     |
| 2           | 6-COOCH <sub>2</sub> H <sub>5</sub> | C <sub>2</sub> H <sub>5</sub>    | N-CH <sub>3</sub>             | 6-COOCH <sub>2</sub> H <sub>5</sub>                          | C <sub>2</sub> H <sub>5</sub>   | N-CH <sub>3</sub>                | H                 | I <sup>-</sup>                                | 2              | 7                  | 516              |     |
| 3           | 5-SO <sub>2</sub> CF <sub>3</sub>   | C <sub>2</sub> H <sub>5</sub>    | N-CH <sub>3</sub>             | 5-SO <sub>2</sub> CF <sub>3</sub>                            | C <sub>2</sub> H <sub>5</sub>   | N-CH <sub>3</sub>                | H                 | I <sup>-</sup>                                | 2              | 6                  | 520              |     |
| 4           | 5,6-dICl                            | C <sub>2</sub> H <sub>5</sub>    | N-CH <sub>3</sub>             | 5,6-dICl                                                     | C <sub>2</sub> H <sub>5</sub>   | N-CH <sub>3</sub>                | H                 | I <sup>-</sup>                                | 2              | 6                  | 516              |     |
| 5           | 5,6-dICl                            | C <sub>2</sub> H <sub>5</sub>    | N-CH <sub>3</sub>             | 5,6-dICl                                                     | C <sub>2</sub> H <sub>5</sub>   | N-CH <sub>3</sub>                | H                 | I <sup>-</sup>                                | 2              | 4                  | 534              |     |
| 6           | 6-Cl                                | CH <sub>2</sub> -CH <sub>3</sub> | C <sub>2</sub> H <sub>5</sub> | N-CH <sub>3</sub>                                            | CH <sub>2</sub> CH <sub>3</sub> | C <sub>2</sub> H <sub>5</sub>    | N-CH <sub>3</sub> | H                                             | I <sup>-</sup> | 2                  | 6                | 501 |
| 7           | 5,6-diBr                            | CH <sub>2</sub> -CH <sub>3</sub> | C <sub>2</sub> H <sub>5</sub> | N-CH <sub>3</sub>                                            | 5,6-diBr                        | C <sub>2</sub> H <sub>5</sub>    | N-CH <sub>3</sub> | H                                             | I <sup>-</sup> | 3                  | 6                | 623 |
| 8           | 5,6-dICl                            | CH <sub>2</sub> -CH <sub>3</sub> | C <sub>2</sub> H <sub>5</sub> | N-CH <sub>3</sub>                                            | 5,6-dICl                        | C <sub>2</sub> H <sub>5</sub>    | N-CH <sub>3</sub> | H                                             | I <sup>-</sup> | 3                  | 5                | 636 |
| 9           | 5,6-dICl                            | CH <sub>2</sub> -CH <sub>3</sub> | C <sub>2</sub> H <sub>5</sub> | O                                                            | 5,6-dICl                        | C <sub>2</sub> H <sub>5</sub>    | O                 | CH <sub>3</sub> COO <sub>2</sub> <sup>-</sup> | 1              | 4                  | 494              |     |
| 10          | 5,6-dICl                            | CH <sub>2</sub> -CH <sub>3</sub> | C <sub>2</sub> H <sub>5</sub> | O                                                            | 5,6-dICl                        | C <sub>2</sub> H <sub>5</sub>    | O                 | CH <sub>3</sub> COO <sub>2</sub> <sup>-</sup> | 1              | 4                  | 496              |     |
| 11          | 6-Cl                                | CH <sub>2</sub> -CH <sub>3</sub> | C <sub>2</sub> H <sub>5</sub> | O                                                            | 6-Cl                            | CH <sub>2</sub> -CH <sub>3</sub> | O                 | CH <sub>3</sub> COO <sub>2</sub> <sup>-</sup> | 1              | 5                  | 491              |     |
| 12          |                                     | CH <sub>2</sub> -CH <sub>3</sub> | C <sub>2</sub> H <sub>5</sub> | O                                                            |                                 | CH <sub>2</sub> -CH <sub>3</sub> | O                 | CH <sub>3</sub> COO <sub>2</sub> <sup>-</sup> | 1              | 4                  | 493              |     |
| 13          | 5,6-dICl                            | CH <sub>2</sub> -CH <sub>3</sub> | C <sub>2</sub> H <sub>5</sub> | O                                                            | 5,6-dICl                        | C <sub>2</sub> H <sub>5</sub>    | O                 | CH <sub>3</sub> COO <sub>2</sub> <sup>-</sup> | 1              | 4                  | 490              |     |
| 14          | 5-CN                                | CH <sub>2</sub> -CH <sub>3</sub> | C <sub>2</sub> H <sub>5</sub> | O                                                            | 5-CN                            | C <sub>2</sub> H <sub>5</sub>    | O                 | CH <sub>3</sub> COO <sub>2</sub> <sup>-</sup> | 1              | 6                  | 495              |     |
| 15          | 5,6-dICl                            | CH <sub>2</sub> -CH <sub>3</sub> | C <sub>2</sub> H <sub>5</sub> | O                                                            | 5,6-dICl                        | C <sub>2</sub> H <sub>5</sub>    | O                 | CH <sub>3</sub> COO <sub>2</sub> <sup>-</sup> | 1              | 6                  | 495              |     |
| 16          |                                     | CH <sub>2</sub> -CH <sub>3</sub> | C <sub>2</sub> H <sub>5</sub> | NCH <sub>3</sub>                                             | 5,6-dICl                        | C <sub>2</sub> H <sub>5</sub>    | O                 | CH <sub>3</sub> COO <sub>2</sub> <sup>-</sup> | 1              | 7                  | 500              |     |
| 17          | 5-SO <sub>2</sub> CF <sub>3</sub>   | OCH <sub>3</sub>                 | NCH <sub>3</sub>              | 5,6-dICl                                                     | OCH <sub>3</sub>                | NCH <sub>3</sub>                 | O                 | H                                             | 1              | 5                  | 504              |     |
| 18          |                                     | OCH <sub>3</sub>                 | NCH <sub>3</sub>              | 5-C <sub>4</sub> H <sub>9</sub> SO <sub>3</sub> <sup>-</sup> | OCH <sub>3</sub>                | NCH <sub>3</sub>                 | NCH <sub>2</sub>  | H                                             | 1              | 7                  | 506              |     |

TABLE B



| Test No. | Z                                                                                   | Y                                                     | R                                                                     | X                       | Steps | Sens. max. (nm.) |
|----------|-------------------------------------------------------------------------------------|-------------------------------------------------------|-----------------------------------------------------------------------|-------------------------|-------|------------------|
| 1        |    | $\text{CH}-\text{CH}=\text{CH}-\text{C}(\text{CH}_3)$ | $-\text{CH}(\text{CH}_2\text{CH}_2\text{CH}_3)\text{CH}_2\text{CH}_3$ | S                       | 6     | 598              |
| 2        |    | $\text{CH}-\text{CH}$                                 | $\text{C}_2\text{H}_5$                                                | S                       | 7     | 480              |
| 3        |    | $\text{CH}-\text{CH}$                                 | $\text{CH}_3$                                                         | $\text{NCH}_3$          | 9     | 468              |
| 4        |   | $\text{OH}-\text{CH}$                                 | $\text{CH}_3$                                                         | $\text{NO}_2\text{H}_5$ | 11    | 480              |
| 5        |  | $\text{CH}-\text{CH}$                                 | $\text{CH}_3$                                                         | $\text{NC}_2\text{H}_5$ | 12    | 480              |

TABLE G



| Test No. | Z | R <sub>1</sub>                                 | Sensi-tivity<br>max:<br>(nm.) | First<br>visible<br>step |
|----------|---|------------------------------------------------|-------------------------------|--------------------------|
| 1        |   | N(C <sub>2</sub> H <sub>5</sub> ) <sub>3</sub> | 420                           | E                        |
| 2        |   | N(C <sub>2</sub> H <sub>5</sub> ) <sub>3</sub> | 420                           | E                        |
| 3        |   | N(CH <sub>3</sub> ) <sub>3</sub>               | 398                           | E                        |
| 4        |   | N(CH <sub>3</sub> ) <sub>3</sub>               | 396                           | E                        |
| 5        |   | N(CH <sub>3</sub> ) <sub>3</sub>               | <400                          | E                        |

45

Table C—Continued

| Test No. | Z                                                                                    | R <sub>1</sub>                                     | Sensitivity max. (nm.) | First visible step |
|----------|--------------------------------------------------------------------------------------|----------------------------------------------------|------------------------|--------------------|
| 6.....   |  | N(CH <sub>2</sub> CH <sub>2</sub> Cl) <sub>3</sub> | 400                    | 6                  |
| 7.....   |  | N(CH <sub>2</sub> CH <sub>2</sub> CN) <sub>3</sub> | 400                    | 6                  |

**60 We claim:**

1. A method of recording information comprising the steps of (1) imagewise exposing to activating electro-magnetic radiation a photosensitive recording element comprising a photo-oxidizing biimidazolyl compound that stands in chemically reactive contact with a compound having reducing properties, which properties are destroyed by a reaction in the exposed areas of the element with the photo-oxidized bi-imidazolyl compound, (2) uniformly contacting the thus-exposed element with an image-forming compound reactive on heating with said reducing compound to produce a distinctive coloration, and (3) heating the exposed element while in contact with said image-forming compound to produce a visible image corresponding to the unexposed areas of said element by reaction of the reducing compound in said areas

25

with said image-forming compound, said biimidazolyl compound having the general formula:



wherein: each of R<sub>1</sub>, R<sub>2</sub> and R<sub>3</sub> stands for a carbocyclic or heterocyclic group with aromatic character, said group being free from Zerewitinoff hydrogen atoms and each dotted line circle represents 4 delocalized electrons, and said compound having reducing properties is selected from:

- (1) aromatic polyhydroxyl compounds and oxidizable derivatives thereof;
- (2) aromatic polyamino compounds and oxidizable derivatives thereof;
- (3) aromatic hydroxyl-amino compounds and oxidizable derivatives thereof; and
- (4) compounds of the general formula:



wherein:

X represents oxygen, sulphur, -NH-, -CH<sub>2</sub>-, -CH=CH-, or



and

Z<sub>1</sub> and Z<sub>2</sub> each represent the necessary atoms to close a carbocyclic aromatic ring.

2. The method of claim 1 wherein said image-forming compound is uniformly carried on an image-receiving element which is brought into contact with said exposed recording element and upon heating of said exposed element, said reducing compound is transferred from the unexposed areas thereof to said image-receiving element and reacts with the image-forming compound thereon to produce said visible image.

3. The method of claim 1 wherein said reducing compound and said image-forming compound are carried in separate layers on said recording element and upon heating of said element are brought into reactive contact.

4. A method according to claim 1 wherein the biimidazolyl compound corresponds to one of the following isomeric structures:



wherein the R<sub>1</sub>, R<sub>2</sub> and R<sub>3</sub> groups have an aromatic character, and any substituents on these groups are free from Zerewitinoff hydrogen atoms.

5. A method according to claim 1 wherein the biimidazolyl compound corresponds to the following general formula:



26

wherein the valencies of the atoms in the imidazolyl rings, other than those joining the imidazolyl rings, are satisfied by two conjugated intracyclic double bonds, and wherein A is a substituted phenyl radical of the formula:



10

wherein R<sub>1</sub> represents a substituent free from active hydrogen atoms and R<sub>2</sub>, R<sub>3</sub> and R<sub>4</sub> represent hydrogen or substituents free from active hydrogen atoms or two in adjacent positions taken together form a benzo ring, with the proviso that any substituent ortho to the imidazolyl radical has a sigma constant below 0.7; and B and D are phenyl groups which are unsubstituted or substituted with up to three substituents free from active hydrogen atoms,

20 two of which, in adjacent positions on the phenyl ring, may together form a benzo ring; with the proviso that at least one of the ortho positions in each of the phenyl groups B and D is unsubstituted.

6. A method according to claim 5 wherein the substituents on the phenyl radicals A, B and D are each in alkyl group containing up to six carbon atoms, an alkoxy group containing up to six carbon atoms, a chlorine, bromine or fluorine atom, or on adjacent pairs form together a benzo ring.

25 7. A method according to claim 1 wherein said compound having reducing properties is volatile between 60 and 200° C.

8. A method according to claim 7 wherein said reducing compound is a phenol or naphthol.

30 9. A method according to claim 8 wherein said reducing compound is a phenol or naphthol having at least two hydroxyl groups directly bonded to the aromatic ring or an ether thereof.

40 10. A method according to claim 1 wherein said reducing compound is an aromatic hydroxyl-amino compound of the benzene or naphthalene series in which compound a hydroxyl group and an amino group are present in ortho- or para-position.

45 11. A method according to claim 10 wherein the photo-oxidizable compound is 4-methoxy-1-naphthol.

12. A method according to claim 1 wherein the biimidazolyl compound has been spectrally sensitized.

50 13. A method according to claim 2 wherein the receiving material comprises a substantially non-light-sensitive noble metal salt.

14. A method according to claim 13 wherein the noble metal salt is a silver salt of an aliphatic carboxylic acid having from 8 to 24 carbon atoms.

55 15. A method according to claim 14 wherein the silver salt is silver behenate.

16. A photosensitive recording material containing a bi-imidazolyl compound, and in chemically reactive contact with said compound (1) a phenol or naphthol having at least two hydroxyl groups directly bonded to the aromatic ring or an ether of said phenol or naphthol, or (2) an aromatic hydroxyl-amino compound of the benzene or naphthalene series, in which a hydroxyl group and an amino group are present in ortho- or para-position, said bi-imidazolyl compound corresponding to the general formula:



70

wherein:

each of R<sub>1</sub>, R<sub>2</sub> and R<sub>3</sub> stands for a carbocyclic or heterocyclic group with aromatic character and each dotted line circle stands for 4 delocalized electrons.

75

17. A photosensitive recording material according to claim 16 wherein the photo-oxidizable compound is 4-methoxy-1-naphthol.

18. The recording method of claim 1 wherein said bi-imidazolyl compound is present in said element in the amount of about 0.5-2 g./sq. m. and said reducing compound is present in a ratio relative to said bi-imidazolyl compound of about 1:2-5 on a molar basis.

19. The recording material of claim 16 wherein said bi-imidazolyl compound is present in said element in the amount of about 0.5-2 g./sq. m. and said reducing compound is present in a ratio relative to said bi-imidazolyl compound of about 1:2-5 on a molar basis.

## References Cited

## UNITED STATES PATENTS

|             |        |                 |          |
|-------------|--------|-----------------|----------|
| 3,445,234   | 5/1969 | Cescon et al.   | 96—90    |
| 3,585,038   | 6/1971 | Cescon et al.   | 96—90    |
| 5 2,789,904 | 4/1957 | Benbrook et al. | 96—49    |
| 3,531,286   | 9/1970 | Renfrew         | 96—114.1 |

NORMAN G. TORCHIN, Primary Examiner

10 W. H. LOWE, Jr., Assistant Examiner

U.S. CL. X.R.

96—88, 49, 77; 117—36.2